

Aug. 27, 1935.

A. G. BROWN ET AL

2,012,805

PROCESS OF MAKING INSULATION BOARD

Original Filed Jan. 25, 1932 2 Sheets-Sheet 1



Aug. 27, 1935.

A. G. BROWN ET AL

2,012,805

PROCESS OF MAKING INSULATION BOARD

Original Filed Jan. 25, 1932 2 Sheets-Sheet 2



Inventors

Alfred G. Brown  
Stephen E. McPartlin

By  
Lorraine  
and Van Autry  
Attorneys

## UNITED STATES PATENT OFFICE

2,012,805

## PROCESS OF MAKING INSULATION BOARD

Alfred G. Brown, Los Angeles, Calif., and Stephen E. McPartlin, Chicago, Ill.

Refiled for application Serial No. 588,538, January 25, 1932. This application November 28, 1934, Serial No. 755,216

7 Claims. (Cl. 18—48)

This invention relates to thermo-insulation material and the process of making the same and is refiled for an abandoned application by the same inventors filed January 25, 1932, Serial No. 588,538. The specific form of the product made in accordance with this invention is a so-called self-sustaining insulating material in slab or board form having considerable rigidity.

Previous methods of producing analogous materials made from fibers necessitated cooking the raw fibrous materials and washing or bearing and mixing the material in large quantities of water, then assembling the material in a machine or in molds and subsequently putting the formed material through a drying process. The present invention does not involve cooking or moistening the fibrous material and therefore eliminates both the steps of cooking and moistening and also drying which were necessary in the previously known methods.

The present invention provides a self-sustaining insulating material which is extremely light in weight, water-proof and which has a high thermo-insulating efficiency. The production is manufactured from a fibrous material such as preferably rice straw or rye straw or a mixture of the two, such containing practically no food value and being a waste product and therefore cheap and readily available in large quantities. The fibrous material had many air cells in its structure which are sealed by a water-proof impervious coating such as preferably an asphalt composition applied during the manufacturing process and the fibers are entwined during the process and formed into a flat board shape while heat is applied and when cooled the asphalt coating serves as an adhesive to rigidly join the fibers in their entwined condition, thus producing many air cells in the structure of the product outside of the air cells in the fibers themselves which have been sealed by the asphalt coating.

The invention conceives a novel method of manufacture which involves shredding straw into its fine component fibers, heating the fibrous mass to remove the commercial moisture therefrom, applying a coating of water-proof asphalt composition to the fiber while it is thus heated and dried, forming the fibers into flat board-like shape and congealing the asphalt coating by cooling to retain the shape and consistency of the produce all of which is performed in a most efficient and economical manner and by machinery of relatively low cost which minimizes the cost of the product.

The invention provides various other new and useful features hereinafter more specifically described and particularly pointed out in the claims, reference being had to the accompanying drawings, in which,

Figs. 1 and 2 are respectively the forward and rear portions of a machine adapted to perform the process of manufacture embodying the present invention, said machine being shown in diagrammatic form and the said figures being considered as components of each other.

Fig. 3 is a transverse sectional elevation on the line 3—3 of Fig. 2, and

Fig. 4 is a perspective view of a section of the finished product.

Like reference numbers refer to like parts in all the figures.

The fibrous material from which the present insulating product is to be made is preferably straw such as rice straw or rye straw which is usually obtained in bale form, which bales 1 are placed upon a feeding conveyor 2 which conveys the bales, usually formed in sections 1a, to a separator having a lower moving table 3 and an upper separating belt 4. The table 3, which may be in the form of an endless conveyor, is provided with spikes 3a and moves at a relatively slow speed while the separator 4, which may be of similar construction having spikes 4a, moves at a faster speed thus separating the straw in the sections 1a of the bale, loosening it and moving it forward from where it enters between two sets of feeding rollers 5 and 6.

The feeding rollers 5 and 6 deliver the loosened straw into the picker or shredding machine which comprises a rapidly rotating drum 7 having teeth or spikes 7a projecting from its cylindrical surface and an arcuate member 8 having teeth or spikes 8a projecting from its inner curved surface. The member 8 partially surrounds the cylindrical surface of the drum 7 and its teeth 8a are in staggered relation axially with the teeth of the drum so that the respective teeth 7a and 8a will move past each other as the drum rotates.

The straw, which is fed between the drum and the member 8, is acted upon by the teeth 7a and 8a to comb the straw into lengthwise position and to shred it longitudinally and separate it into its fine component elongated fibers. It may be here stated that the member 8 is adjustable relative to the drum and that the actual picker machine which is here shown in diagram only embodies various details of construction which will enable it to efficiently perform its function, the said ma-

5

10

15

15

15

20

25

30

35

40

45

50

55

55

chine in detail being the subject of another proposed patent application not yet filed.

After the straw has been shredded into fibers the fibers are deposited in a conveyor 9 which is in the nature of a blow-pipe and it is intended that the air current developed by rotation of the drum 7 and directed from its periphery will be of sufficient force to carry the fibers designated as 10 through said blow-pipe conveyor upwardly where they are deposited through a device commonly known as a cyclone separator 11 at the top of a bin 12 and the fibers then dropped by gravity into said bin. It is conceived that additional air current to carry the fibers through the conveyor pipe 9 may be supplied from a suitable source if necessary or another type of conveyor may be substituted for the blow-pipe if desired.

The bin 12 is preferably of considerable capacity and has an appreciable bottom area which is heated by means hereafter described and the heat radiating from the bottom of the bin serves to heat the contents thereof and particularly the fiber closest to the bottom which heat drives off the commercial moisture of the fiber, which has been found to be approximately 9% of the original weight, this moisture being dissipated upwardly and emitted from the bin through its open top.

A conveyor comprising a horizontal shaft 13 upon which are mounted a plurality of paddles 14 inclined relative to the axis of the shaft is located with one of its ends extending into the bottom portion of the bin 12 and projecting therefrom a considerable distance in a trough-like structure 15 which trough has a cover 16. The shaft 13 is rotated by any suitable means such as a belt passing over a pulley 17 and driven by convenient power means, such rotation being at a speed sufficient to agitate and mix the fiber and at the same time carry it forward through the trough 15 in a direction away from the bin 12.

At a point closely adjacent the bin 12 and in a location where the fiber is still in its heated and dry condition and has not come in contact with outside atmosphere the asphalt coating material is applied through a feed pipe 18 which obtains its supply from a heated reservoir 19 provided with a suitable burner 20 by means of which heat is supplied. The asphalt coating substance is preferably a blended mixture of asphalts of relatively high and low melting points one of which may melt at approximately 230° F. while the other at 170° F., to which is preferably added a small quantity, about 2% of the whole, of crude petroleum oil. This coating material is heated to a temperature at which it will flow freely and is deposited in the proper quantity onto the fiber 10 as it is passed through the trough 15 by the conveyor. The trough 15 is heated as hereafter described and is of considerable length so that the paddles 14 of the conveyor while acting to move the fibers to which the asphalt coating has been applied will also thoroughly agitate and mix the mass during its travel through the trough and assure complete coating of all of the fibers with the coating material.

At the termination of the trough 15 a slightly restricted passage 21 is formed through which the coated fibers are forced by action of the conveyor and somewhat compressed in passing through the restricted passage from which they enter a tamping chamber 22 in which reciprocates a tamper 23. The tamper 23 may be moved by any suitable mechanism such as a crank 24 which is driven by desirable means and the speed

of the crank and the accompanying reciprocation of the tamper 23 may be varied relative to the speed of the conveyor shaft 13 with the result that the solidity of the mass compressed by the tamper may be varied.

The tamping chamber 22 emerges at its lower end into a forming and pressure chamber 25 which has a rigid bottom 26 and a top formed by a plate 27 hinged at the entrance side and supported at the outlet side by a turn-buckle 28, which turn-buckle may be adjusted to regulate the position of the movable edge of the plate 27 and thus govern the vertical dimension of the outlet side of the compression chamber 25.

A lower conveyor belt 29, passing over pulleys 30 and also over supporting rollers 31, traverses a horizontal plane from a location immediately following the outlet side of the compression chamber 25 and receives the material emitted from said compression chamber in the form of a continuous flat strip. Two pressure rollers 32 and 33 are located one above the other with their peripheries in spaced relation, the lower roller 32 being located intermediate the length of the conveyor belt 29 with the upper portion of its periphery in engagement with said belt and an upper conveyor belt 34 run over the upper pressure roller 33 and also over a pulley 35 with its lower stretch horizontal and parallel with and spaced above the upper stretch of the belt 29. Supporting rollers 36 engage the lower horizontal stretch of the belt 34 to hold it in its proper position. The material traveling upon the conveyor belt 29 will be passed between said belt 29 and the upper belt 34 and will be compressed between the rollers 32 and 33.

It is desirable to apply a paper covering to the upper and lower surface of the material, which paper covering is supported from rolls 37 and 38, said paper traveling upon the surfaces of the respective belts 29 and 34 and coming in contact with the material and adhering thereto as the material passes between the belts. After leaving the belts 29 and 34 the material with its paper covering is passed between upper and lower series 40 of retaining rollers 39 and 40 which are located in atmosphere at room temperature which permits the material to cool while being passed between said rollers.

The portions of the device in which the fiber is coated, mixed, conveyed, tamped and formed are heated by suitable means such as a burner 41 located beneath a baffle plate 42 and the heated air therefrom is directed around the compression chamber 25 and the rollers 32 and 33 a small portion of it being emitted through a stack 43 causing a constant flow of highly heated air around the said parts and the remainder of the heated air flows toward the forward part of the machine contacting the bottom and sides of the trough 15 and heating the bottom of the bin 12. After serving its purpose the heated air is emitted through a vertical stack 44 which stack is preferably located in contact with a vertical side of the bin 12 and a stack 45 which carries away hot gases from the burner 20 is preferably located adjacent the opposite side of the bin 12 thereby supplying heat to aid in dissipation of moisture from the fiber.

#### Operation

The raw material from which the fibers are obtained is fed into the separator by the conveyor 2 and as previously stated, this raw material is preferably rice straw. Rye straw ap-

proximates rice straw in desirable quality and may be substituted entirely therefor or a mixture of the two may be used. If desired other fibrous material may be substituted for either of the preferred materials, the essence of this invention not being dependent upon a certain specific fibrous substance.

The straw, which has been matted and compressed in bales, enters the separating device comprising the slowly moving table or conveyor 3 and the more rapidly moving belt 4 which loosen the straw and feed it in its loosened condition between the sets of feed rollers 5 and 6 from where it is delivered against the periphery of the rapidly rotating drum 7 of the picker device. The teeth on the surface of the picker, coacting with the teeth of the stationary arc-shaped member 8, pull the straws into longitudinal position and shred them lengthwise into their component fine fibers, the picker being designed and acting to break the straw and fibers as little as possible.

After the straw has thus been shredded into fibers, the fibers are deposited in the bin 12 by means of the blow-pipe conveyor 9 or other suitable conveying means and the fibers drop by gravity to the bottom of the bin and pile therein to a height depending upon the amount of fibers deposited in the bin relative to the amount removed therefrom.

The bottom of the bin is heated by means heretofore described and also the sides of the bin are preferably heated to some extent and this heat serves to drive off by evaporation the commercial moisture contained in the fibers which amounts to approximately 9% of the weight thereof, the evaporated moisture being exhausted from the open top of the bin.

The fibers thus substantially dried and heated are removed from the lower part of the bottom of the bin adjacent its heated bottom by the combined conveyor and mixer immediately after leaving the bin and while dry and heated and before being exposed to normal atmosphere a coating substance is applied to the fibers. The coating substance is preferably an asphalt composition which solidifies at normal temperatures and which has been heated sufficiently to cause it to flow readily. The coating material is supplied through the pipe 18 and its volume or rate of flow may be controlled by a valve 18a in the pipe.

The fibers with the heated fluid coating material are conveyed through the trough 15 by rotation of the shaft 13 with its paddles 14 thereon, the said paddles serving to gradually move the fibers forwardly in the trough and at the same time thoroughly agitate the fibrous mass which has been mixed with the coating material so that during travel through the trough each of the fibers is certain to obtain a thorough covering of the coating material. The trough is heated and its contents are maintained in heated condition during the conveying and agitating process to prevent congealing of the coating material.

After the fibers and coating material have been thoroughly mixed they are ejected from the trough into the slightly restricted passage 21 which serves to compress the mass to some extent and from the passage 21 the slightly compressed mass is moved into the tamping chamber 22 where the mass is acted upon and further compressed by the reciprocating tamper 23. The tamper 23 in addition to its compressing function also moves the mass forwardly through the compression chamber 25 where the mass is further compressed, the amount of such compres-

sion depending upon adjustment of the top plate 27 and the vertical dimension of the outlet opening between the plate 27 and the fixed plate 26 and this vertical dimension is substantially the thickness of the finished product.

It may here be explained that the density of the finished product or the amount of compression to which it is submitted is not governed entirely by adjustment of the plate 27 but is also regulated by the speed of the conveying device 10 relative to the speed of the tamper. If the conveying device is run at a relatively high speed, which will cause a considerable amount of the fibrous mass to be fed into the tamping chamber between each reciprocation of the tamper, then the tamper will compress the mass in the tamping chamber to a greater extent than it would if a smaller amount of fibrous material were fed between each of the tamper's reciprocations and this greater compactness of the substance is carried on through the compression chamber and the resulting product will be relatively dense in texture.

The compressed material of substantially uniform thickness emitted from the compression chamber is deposited upon the conveyor belt 29 over which is spread the paper supplied by the roll 31 which paper serves as a covering for one side of the finished product and immediately thereafter the material passes under the belt 34 30 which likewise has been supplied with paper from the roll 38 and this paper serves as a cover for the opposite side of the finished product. While passing between the belts 29 and 34, the material is submitted to a slight further compression 35 as it passes between the rolls 32 and 33 which serves more in the nature of a finishing pressure than to actually increase the density of the product and the thickness of the product is accurately regulated by said rolls.

Following the rolls 32 and 33 the material continues between the belts 29 and 34, which are supported by the rollers 31 and 36, and after leaving the said belts the product with the paper covering adhering to its upper and lower sides passes 45 between series of upper and lower cooling rollers 39 and 40, said cooling rollers being located outside of the heated portion of the machine and in ordinary atmospheric temperature.

The material continues between said cooling 50 rollers for a distance sufficient to permit the asphalt coating substance to congeal and permanently secure the mass in rigid board-like form and the continuous strip of material emerging from the machine is cut off by suitable means 55 into convenient lengths for handling.

The foregoing description has described a machine having a single conveyor and tamper and associated parts and such a construction would be operative and suitable for a product of relatively narrow width. However, the ordinary commercial product would be of width greater than could be effectively produced by a single set of the devices mentioned and therefore said devices may be duplicated side by side in numbers 60 sufficient to produce a board of desired width and in actual practice the number of sets of the device will be varied in accordance with the width of the product to be made.

The product thus formed is in the nature of a 70 slab or board of desirable width and thickness, both of which dimensions may be altered as desired and the article has considerable rigidity which makes it of the self-sustaining class.

The substance comprising the board consists of 75

innumerable fibers, each of which contains its natural air cells, the moisture having been substantially removed therefrom and the fibers all thoroughly coated with a water-proof asphalt composition so that the air cells in each of the fibers have been thoroughly sealed and the fibers are impervious to moisture. The structure also contains innumerable air cells formed between the fibers which are interlaced in a manner to form such air cells and the same coating substance when cool joins the fibers to each other by its adhesive quality and also effectively seals the air cells or spaces between the fibers making them also substantially impervious to moisture. The solidified coating forms the whole mass into a rigid structure and also serves to adhere the paper covering to its respective broad sides.

Thus the product constitutes a water-proof material of high thermo-insulating value, the sealed air cells in the structure combined with the non-conductivity of the material itself serving to resist the transmission of heat. Actual tests have shown the substance to be at least equal in thermal insulating value to compressed cork which is a standard of measure and the cost of the product is greatly less than that of cork or any other known insulating substance of analogous quality.

The machine involved in manufacturing the product in accordance with this invention is relatively simple and inexpensive as compared with the machinery necessary to manufacture other thermo-insulating materials of analogous qualities and therefore the cost of the product is very greatly reduced.

The invention is defined in the appended claims and is to be considered comprehensive of all forms of structure coming within their scope.

We claim:

1. The process of making insulating material comprising, depositing a mass of separated fibers in a container which is heated sufficiently to dissipate the commercial moisture in the fibers, conveying said fibers from said container while in dried state through a heated conveyor, applying a heated coating material to said fibers in said conveyor, said coating material being liquid while heated and solid at ordinary temperatures, agitating said mass of fibers and coating material in said conveyor sufficiently to cause such fiber to become coated with said coating material, intermittently subjecting said agitated mass to pressure, and then gradually applying pressure thereto while said coating material hardens.

2. The process of making insulating material comprising, providing a quantity of separated fibers, conveying said fibers along a heated conveyor, applying a heated coating material to said fibers in said conveyor, said coating material being liquid while heated and solid at ordinary temperatures, agitating said mass of fibers and coating material in said conveyor sufficiently to cause each fiber to become coated with said coating material, intermittently subjecting said agitated

mass to pressure, and then gradually applying pressure thereto while said coating material hardens.

3. The process of making insulating board comprising, shredding a mass of fibers, then heating the mass of separated fibers to a temperature at which moisture therein will be dissipated, applying water-proof adhesive coating material to said fibers while in their dried and heated stage, then mixing the fibers so that they are positioned irregularly to one another, and then forcing the fiber mass so coated into a product of desired shape.

4. The process of manufacturing comprising, providing a quantity of separated fibers, applying coating and adhesive material to said fibers, mixing the fibers so that the fibers are located angularly to each other whereby a relatively great percentage of voids is attained, and then subjecting the mixture to pressure of predetermined intensity to reduce the percentage of voids as desired.

5. The process of making insulating board or the like comprising, confining and heating a mass of separated fibers of straw to a temperature at which ordinary commercial moisture therein will be dissipated, applying water-proof coating material to said fibers while in their dried state, bending and then forming the fiber mass so coated into a product of desired shape.

6. The process of making an insulating material comprising, heating a mass of separated fibers to a temperature at which the moisture therein will be dissipated, maintaining the same against contact with cold air, applying the asphalt composition coating to said fibers while in such dried and heated state, said coating material being water-proof and solidified at ordinary temperatures and being applied to said fibers while heated sufficiently to be liquid, mixing the fibers so as to cause an appreciable size in their bulk and finally forming said mass of coated fibers into a product of desired shape while in heated condition and cooling said formed mass to permit said coating material to solidify and thereby retain the mass in desired form.

7. The process of making insulating material comprising, shredding a fibrous straw material into its component individual fibers, submitting said separated fibers to heat sufficient to dissipate the commercial moisture therefrom, applying a heated water-proof adhesive coating material to said fibers while they are in dried and heated state, agitating said fibers under a minimum of pressure, said coating material being fluid when heated and solid at normal temperatures, and said coating material being applied in a manner to thoroughly coat each separate fiber and then forming the coated fibrous mass into desired shape.

ALFRED G. BROWN.  
STEPHEN E. McPARTLIN.